

Patented Sept. 21, 1937

2,093,464

# UNITED STATES PATENT OFFICE

2,093,464

## CELLULOSE ESTERS CONTAINING SUC- CINYL GROUPS AND PROCESS OF MAK- ING SAME

Carl J. Malm, Rochester, N. Y., and Charles E. Waring, Dayton, Ohio, assignors, by mesne assignments, to Eastman Kodak Company, Jersey City, N. J., a corporation of New Jersey

No Drawing. Application July 30, 1932,  
Serial No. 627,150

11 Claims. (Cl. 260—101)

The present invention relates to the succinic acid esters of cellulose and the preparation of the same by reacting upon a cellulosic material with succinic anhydride in the presence of an organic base.

This application is a continuation in part of our U. S. application Serial No. 380,252 filed July 22, 1929 in which there is described and claimed the preparation of dicarboxylic acid esters of cellulose by reacting upon cellulosic materials with the corresponding anhydride of the acid in the presence of an organic base.

In U. S. Patent No. 1,704,306 of Stinchfield is disclosed a process of preparing phthalyl containing cellulose esters. In that process one of the carboxyl groups of the phthalic acid must be esterified before the phthalic acid can be impelled into the cellulose. There is no disclosure in that patent of the preparation of succinic acid esters in any manner. There are other instances in the prior art of treatment of cellulose with phthalic compounds but nowhere have succinates been described as being prepared. Whether or not either of the above processes using succinic instead of phthalic compounds would be operable is immaterial as even if those processes could be employed for the preparation of succinic esters of cellulose they would possess disadvantages which are overcome in our process of preparing succinic acid esters of cellulose.

One object of our invention, therefore, is to provide a process for producing succinic acid esters of cellulose and more particularly a process in which the esterification takes place in one step, thus eliminating the necessity of preliminarily esterifying one of the carboxyl groups of the succinic acid before the esterification of the cellulosic material occurs. Another object of our invention is to produce a succinic acid ester of cellulose which is soluble in a number of the organic solvents commonly employed for dissolving and preparing commercial products from cellulose esters. Another object of our invention is to provide a process for the dope succinylation of cellulose rather than the mere superficial succinylation of cellulose fibers. Other objects will hereinafter appear.

We have found that cellulose esters of succinic acids can be readily formed by treating cellulosic materials with a substantial amount of succinic anhydride in the presence of an organic base. We have found that by this reaction the cellulosic material is esterified by only one of the two carboxyl groups and that the other carboxyl group combines during the reaction with the organic base from which it can be later freed if desired by treating the resulting compound with comparatively strong acid such as the mineral acids.

We have found that by reacting upon cellulose

with a substantial amount of succinic anhydride in the presence of an organic base, that up to three molecules of succinic acid may combine with every  $(C_6H_{10}O_5)$  group of the cellulose, which cellulose group will hereinafter be referred to as 5 a unit of cellulose. We have found that by our process we obtain a succinic acid ester of cellulose in dope form, which is the usual form in which cellulose esters are prepared commercially, instead of obtaining a mere superficially succinylated fibrous product which is obtained according to the disclosure of a method of preparing succinic acid esters of cellulose which has recently come to our attention.

We have found that the esters prepared according to our invention especially when a partially hydrolyzed cellulose acetate is employed as the starting material may be formed into products of great commercial value.

Where the term cellulosic material is employed 20 herein it is to be understood as including both esterifiable celluloses such as cotton fibers and linters, paper or any customary types of purified cellulose and the esterifiable cellulose derivatives such as cellulose nitrates, ethers, acetates or 25 acylates having free and esterifiable hydroxyl groups.

The time of the succinylation of cellulosic material is governed to a great extent by the kind of cellulosic material used as the starting material. 30 For example at a temperature of 60–65° C. if unmodified cellulose is employed as the starting material, succinylation may take two or three weeks; while with a cellulose ether containing about 35% ethoxy the time of succinylation may 35 be cut down to about 24 hours. The time of succinylation, however, also depends on other factors such for instance as the temperature. In our invention we have found it generally desirable to carry out the reaction at a temperature below approximately 110° C. but it will be understood that higher or lower temperatures may be used. At the higher temperatures the succinylation will take place in much less time; however, it is desirable that the temperature be kept sufficiently low 40 to insure that a product will not be obtained, the properties of which have been markedly affected by the degradation of the cellulose.

When the required degree of esterification has occurred the succinic ester formed is precipitated 50 by pouring the reaction mass into a dilute mineral acid solution or into an organic non-solvent for the ester such as an alcohol or an ether, for instance isopropyl ether, the latter having been disclosed and claimed in Malm and Fordyce application Serial No. 553,646, filed July 28, 1931.

The succinic esters which are obtained by the process of our invention are generally soluble in various pyridine combinations such as pyridine and water, pyridine and benzene, pyridine and 60

tetrachlorethane, pyridine and ethylene chloride, etc. Any of the latter three combinations may be employed in the succinylation process of our invention instead of using pyridine entirely.

5 Various inert organic solvents may also be em-  
ployed for dissolving the succinic esters, such as  
acetone, methyl alcohol-acetone, methyl acetate,  
ethyl acetate, ethylene chloride-methyl alcohol,  
propylene chloride-methyl alcohol, 1.4 dioxan, B.  
10 methoxyethyl alcohol, ethylene glycol monoace-  
tate, B.B'dichlorethyl ether-methyl alcohol.  
From a solution of a succinic ester of cellulose in  
one of the above-named solvents, a transparent  
sheet or skin may be formed by spreading the so-  
15 lution on a film-forming surface, such as a pol-  
ished drum, and coagulated or solidified in a fluid  
stream of heated air or a non-solvent liquid.  
Various plasticizers such as methyl, ethyl or butyl  
20 phthalate, triphenyl or tricresyl phosphate, mono-  
chloronaphthalene, beta methoxy- or beta ethoxy-  
ethyl phthalate or tributyl phosphate may be  
added to the solution prior to the formation of the  
skins or sheets. These succinic esters of cellu-  
25 lose may also be employed in adhesives, laminated  
glass, lacquers, artificial silk, molded products  
either alone or mixed with a plasticizer and other  
desired addition products. If a molded product  
is desired plasticizers such as B.methoxy ethyl  
30 phthalate which plasticizer is disclosed and  
claimed in Noller application Serial No. 504,640  
filed December 24, 1930 or tributyl phosphate  
which plasticizer is disclosed and claimed in Smith  
application Serial No. 501,667 filed December 11,  
35 1930 are eminently suited as agents of addition to  
the succinic esters especially the acetate-succi-  
nates as these plasticizers have been found to be  
solvents of those cellulose esters at elevated tem-  
peratures.

The following examples are illustrative of the carrying out of our invention:

*Example 1.*—5 gms. of cellulose such as tissue paper was treated with about 25 gms. of succinic anhydride in 75 cc. of pyridine at 60–65° C. the temperature being maintained constant by employing a jacketed container. In about a week a viscous dope was formed. This dope was precipitated in 5% hydrochloric acid and the precipitate was washed and dried. The cellulose succinate formed contained approximately 62% succinyl. Theoretically a fully esterified cellulose trisuccinate contains 65% succinyl.

*Example II.*—10 grams of ordinary commercial acetone-soluble cellulose acetate containing approximately 39% acetyl, was dissolved in 55 cc. of 55 pyridine containing 10 gms. of succinic anhydride and was maintained at a temperature of 60°–65° C. in a jacketed kettle for about 4 days. The

1.4 dioxan, **B**.methoxy ethyl alcohol, ethylene glycol monoacetate and **B**.**B**'dichlorethyl ether-methyl alcohol (4:1). At elevated temperatures this cellulose acetate succinate was found to be soluble in the above solvents and also in methyl alcohol-acetone (2:1, 3:1 and 4:1), benzene-methyl alcohol (1:1) and **B**ethoxy ethyl alcohol. As was pointed out above mixtures of pyridine with benzene, tetrachlorethane or ethylene chloride are solvents of the esters prepared by our invention, consequently a portion of the pyridine or the organic base employed in the esterification bath may be replaced by one or more of these liquids. 10

Instead of pyridine other organic bases, particularly of the tertiary variety may be employed in the process of our invention. In addition to pyridine other bases such as quinoline and alpha picoline have been found to be useful in the process of our invention. Other organic bases such as the dialkyl anilines for instance dimethyl aniline, the hexahydro-dialkyl anilines, dimethyl n-hexylamine and the like would at once suggest themselves to those skilled in the art, as a group which would supply organic bases suitable for employment as the acylating medium in the present invention. 15 20 25

In the process of our invention we have reason to believe that the succinic esters of cellulose prepared therein are combined with the organic base employed in the succinylation. We believe that one of the carboxyl groups of the succinic acid is combined with the cellulose molecule, while the other carboxyl group is combined with the organic base, for example pyridine. While these esters containing pyridine (or another base) in combination may have properties fitting them for particular uses, we find it desirable to treat the succinic esters, we obtain, with an excess of an acid which will free the succinic acid ester of cellulose from the combined pyridine. Although an organic acid such as acetic acid may be employed for this purpose, we prefer to employ a mineral acid. A common mineral acid such as sulfuric, hydrochloric, etc., is preferably employed. 30 35 40 45

The reactions which are believed to take place in the process of our invention may be represented as follows:



in which



is employed to represent one unit of a partially de-esterified cellulose acetate based on  $C_6H_{10}O_5$  as representing a unit of cellulose. Although the proportion of two acetyl groups to 75

